

**1**

3,372,119

**LUBRICANT COMPOSITIONS CONTAINING POLY-CHLOROALKYL BENZENE EXTREME PRESSURE ADDITIVES**

Bernard Demoures, 14 Quai Jayr, Rhone, France, and Gérard Schneider, 119 Quai Clemenceau, Rhone, Caluire, France

No Drawing. Filed Mar. 9, 1965, Ser. No. 438,368  
Claims priority, application France, Mar. 10, 1964,

966,777

4 Claims. (Cl. 252—48.8)

**ABSTRACT OF THE DISCLOSURE**

A lubricant additive for use at extreme pressures comprising a mixture of a chlorinated alkyl benzene having a chlorine content of from 50 to 75% by weight, at least 75% of which is bound to the alkyl carbon atoms, and a resinous polychlorobenzene polysulfide soluble in hydrocarbon oils and containing from 15 to 25% sulfur and from 44 to 55% chlorine.

The present invention relates to new additives for lubricants and in particular to products capable of imparting extreme pressure properties to lubricating oils, making them more suitable for use as cutting oils. It is also concerned with a process for the preparation of these new products.

It is the usual practice to incorporate various adjuvants into lubricants, the purpose of which is to improve the lubricating power, inhibit corrosion, serve as dispersion agents or viscosity-modifying agents, etc. In the very important case of cutting oils, which generally work under very severe conditions of use, it is imperative to employ judiciously selected additives. Actually, when it is subjected to the very high pressures developed on the cutting edge of the tool the lubricating film formed by a normal oil has a tendency to be broken up, thus removing the lubrication at the point where normally it should be applied. The addition of an additive serves the purpose in this case of causing the formation of a second lubricating film which is more resistant than the first, simultaneously on the cutting edge of the tool and on the element in contact with the latter.

A large number of extreme pressure additives have already been proposed and the majority of these are chlorinated derivatives, sulphur or phosphorus derivatives, alone or in combination. Among the chlorinated compounds most employed at the present time, there may be mentioned the chlorinated diphenyls or polyphenyls and particularly the chlorinated paraffins.

It has also been proposed to use chloralkyl benzenes, as for example the 30.5% chlorinated dodecylbenzene, obtained in the form of a reddish brown opaque oil by chlorination of the hydrocarbon in the presence of ultraviolet rays at increasing temperatures which vary between 100 and 220° C.

The new additives according to the invention have an efficiency which is distinctly better than that of the already known chlorinated derivatives, that is to say, the rates of wear of the metal element working under high pressures are comparatively much lower and, in addition, the "seizing" phenomena of the element or tool only occur at very strong pressures which are higher than those corresponding for example, to the chlorinated paraffins. In addition, in view of their very high chlorine content, these additives can be used in very small quantities and, in any case, for identical rates of wear and seizing pres-

**2**

sures, certainly smaller than those of the prior known chloralkyl benzenes.

These additives according to the present invention are formed by aromatic hydrocarbons substituted by one or 5 more chlorinated alkyl radicals, at least one of these radicals containing a minimum of 5 carbon atoms, the total chlorine content in the said hydrocarbons being greater than 50%.

The long-chain alkyl radical may comprise 5 to 30 carbon atoms, it being possible for the aliphatic chain to be linear or branched. The aralkyl hydrocarbons chlorinated by substitution on the side chains and comprising several medium or long chain alkyl radicals on the aromatic nucleus, as well as mixtures of aralkyl hydrocarbons comprising at the same time lower alkyl radicals and at least one alkyl radical with more than 5 carbon atoms, also come within the scope of the invention.

The percentages of chlorine fixed on the aliphatic radical may vary between wide limits and the additives according to the invention may contain in total 50 to 75% of chlorine. The chlorination process according to the invention consists in introducing a current of chlorine into the hydrocarbon or mixture of aromatic alkyl hydrocarbons kept in the dark at a temperature between 40° and 180° C.

The reaction, which is preferably effected in the absence of a solvent, does not generally require the use of a catalyst. Nevertheless, according to a modification of the process according to the invention, it is possible to 20 employ small quantities, for example, 2 to 8% by weight of the batch, of a catalyst which promotes the chlorination of the aralkyl hydrocarbon on the side chain or chains. This catalyst may be formed, for example, by a phosphorus polyhalide, such as phosphorus trichloride. 30 Under these conditions, the reaction temperature can be lowered appreciably and it is then generally between 40° and 100° C.

As initial aralkyl hydrocarbons, it is for example possible to use benzene hydrocarbons substituted by a long-chain alkyl radical, such as: pentyl, hexyl, octyl, nonyl, decyl, dodecyl, tridecyl, tetradecyl, etc. The alkyl radical may in addition be branched, it being possible for one or several hydrogens of the carbon atoms in the linear chain to be substituted by alkyl radicals, such as: 40 methyl, ethyl, propyl, etc. The following may be mentioned as examples of branched alkyl radicals: 2-methyl pentyl, 2,3-dimethyl pentyl, 2-methyl-4-propyl pentyl, 2-ethyl hexyl, 4,6-dimethyl nonyl, etc. Additives which are likewise advantageous are formed by chlorination 45 products of "alkylates" or mixtures of heavy alkylates, obtained at the time of distillation of alkylation products of benzene with branched or unbranched olefins (as for example the tetramer of propylene). As examples, there may be mentioned the alkyl or polyalkyl benzenes known 50 under the registered trademarks: Progiline 152, Solgil 54, Solgil 109, Solgil 110, Alkylat 1163, etc. As stated above, it is also possible to employ mixtures of these products, in which the length of the alkyl chain varies 55 between 5 and 30 carbon atoms.

60 The reaction generally takes place under atmospheric pressure but obviously it is possible to work under higher or lower pressures. It may be conducted continuously or intermittently and it is possible to determine the proportion of fixed chlorine by the usual methods, as for example the measurement of the variations in physical characteristics, such as density, refractive index, etc.

65 The chlorinated products obtained according to the invention are in the form of more or less viscous liquids or solids, which are generally colorless or with a slight yellowish orange coloration. The total proportion of

chlorine therein is preferably between 52 and 60% for the purposes according to the invention.

Although the new additives according to the invention are very efficient, one modification of the invention enables their action to be further strengthened. According to this modification, the effect of the polychloroalkyl aryl compounds on the lubrication is increased in a surprising fashion by the addition of resinous polyhaloaryl polysulphides, which are in themselves agents for improving lubricating oils, but to a lesser degree than when they are employed in conjunction with the polychloroalkyl aryl compounds.

Thus, when one of the polychloroalkyl aryl compounds described above is mixed with a resinous polychloroaryl polysulphide which is soluble in the hydrocarbons and which is referred to in French Patent No. 1,339,529 or No. 1,335,514, it is unexpectedly found that the mixed additive which is formed is more active than is the case with each of its constituents, taken separately. The haloaryl polysulphide employed most usually contains, by weight, 15 to 25% of sulphur and 44 to 55% of chlorine.

The mixed additive in accordance with the modification of the invention may contain variable proportions of each of its constituents, for example, 10 to 90 parts by weight of polychloroalkyl aryl compound to, respectively, 90 to 10 parts of resinous haloaryl polysulphide.

The content of this mixed additive in the lubricants may advantageously be from 2 to 10% by weight.

Although certain chlorinated additives according to the invention are relatively stable over a period of time at normal temperature, others are decomposed more or less quickly from 30° to 40° C., thereby liberating hydrochloric acid. It is possible considerably to limit this degradation by the chlorinated product having incorporated therein one or more heat stabilizers and/or light stabilizers of known types. By way of non-limiting example, the additives may have added thereto: metal salts of fatty acids, such as barium or cadmium laurates and stearates, organo-tin derivatives, epoxidized agents, hydroxybenzophenones, derivatives of alkylene oxide, sulphonamides, morpholines, etc.

Among the stabilizers capable of producing a good stabilization of the chlorinated additives according to the invention up to temperatures of 150° C. and higher, there are to be considered, for example, epoxidized compounds, such as epoxidized soya oil, used at the rate of 1 to 10% of the weight of chlorinated hydrocarbon, alone or admixed with 0.5 to 4% of a hydroxybenzophenone, such as 2-hydroxy-4-methoxybenzophenone.

Furthermore, for improving the resistance to corrosion in the presence of the chlorinated additives, it is sometimes advantageous to incorporate small quantities of corrosion inhibitors of known type, as for example amines or polyamines, mercaptans, alkali compounds, capable of neutralizing the decomposition products which could be formed with the use of the cutting oil.

The quantity of chlorinated additive to be incorporated into a lubricant for permitting it to be used as a cutting oil at extreme pressure is obviously a function of the nature of this lubricant and of the work for which it is intended to be used. This quantity may vary generally between fairly wide limits, for example between 0.2 and 20% of the weight of lubricant. In the case of cutting oils for high pressure, the desirable quantities are frequently between 2 and 10% by weight. It is generally advantageous to use a proportion of additive such that the chlorine content in the lubricating composition is of the order of 1.5 to 4%. It is then found that there is a very great increase in the binding limit and also a considerable reduction in the wear of the tool.

The lubricating oils containing the additives according to the invention may be used for numerous purposes, as for example hypoid drives, motors, cutting of metals, lubrication of drilling bits and rod sections when sinking petroleum wells, etc.

The following examples, given in non-limiting manner, show how the invention can be carried into effect. Examples 1 to 6 illustrate the preparation of a certain number of aralkyl hydrocarbons chlorinated to more than 50% in accordance with the invention. Examples 7 to 14 illustrate the good results obtained when using these chlorinated products as extreme-pressure additives, and also their superiority as compared with previously known chlorinated additives.

The tests of the additives to cutting oils were carried out with the 4-ball Shell machine, particularly described in the journal "Engineering" of July 13, 1933, vol. 136, page 46. The values indicated in the tables for establishing the wear represent the mean of three similar tests.

Unless otherwise indicated, all the percentages are in parts by weight.

#### Example 1

Employed as initial hydrocarbon is a cut of alkylation products of benzene, boiling between 160 and 210° C. and containing a mixture of alkyl benzenes of the mean empirical formula  $C_6H_5C_{6,7}H_{14,4}$ .

410 g. of the aforementioned hydrocarbon are introduced into a two-litre spherical flask kept in the dark and equipped with a stirrer device, a condenser, a gas supply tube and a heating system. Then, after having heated the flask to about 120° C., a stream of chlorine is caused to bubble therein at an average rate of 24 l./hr.

After chlorination for 30 hours at temperatures between 120 and 125° C., followed by nitrogen degasification of the flask, there are obtained 880 g. of a viscous light yellow liquid with a chlorine content of 55.6%.

Analyses of the product, carried out on the spectra of nuclear magnetic resonance and also the infra-red and ultra-violet spectra, made it possible to establish that the chlorination had been effected for the major part (that is to say, to more than 75% of the consumed chlorine) on the alkyl chain of the initial hydrocarbon. The chlorinated product had the characteristics:  $d_4^{20} = 1.460$ ;  $n_D^{20} = 1.5805$ .

#### Example 2

The same equipment and the same initial material as in Example 1 were employed. Starting with 842 g. of hydrocarbon, the chlorination was effected in the dark for 30 hours, keeping the temperature between 150° and 155° C. The rate of flow of chlorine was regulated to a value of about 60 l./hr. for 10 hours, then 48 l./hr. for the following 10 hours, and finally 24 l./hr. during the last 10 hours. After degasifying the flask with nitrogen, there were obtained 1873 g. of an alkyl benzene chlorinated mainly on the chain and in the form of an orange-yellow viscous liquid with a chlorine content of 57.2%. Refractive index:  $n_D^{20} = 1.5914$ . Density =  $d_4^{20} = 1.495$ .

#### Example 3

The operation was carried out with the same equipment and the same initial hydrocarbon as in Example 1, but starting with 274 g. of product, to which had been added 13.7 g. (i.e. 5% by weight) of  $PCl_3$ . By maintaining a chlorine rate of 24 l./hr. for 55 hours and at 50° C. (always in the dark), there were obtained 560 g. of a viscous colorless liquid with a chlorine content of 52.8%. Characteristics:  $d_4^{20} = 1.415$ .  $n_D^{20} = 1.574$ .

#### Example 4

The same initial materials as in Example 3 were used, but with the following proportions and under the following conditions:

70 Weight of hydrocarbon \_\_\_\_ 322 g.  
Weight of  $PCl_3$  \_\_\_\_ 10 g. (3% by weight).  
Rate of flow of chlorine \_\_\_\_ 36 l./hr. for 12 hours, then 24 l./hr. for 12 hours.  
Temperature \_\_\_\_ 90 to 100° C.

75 After degasifying the reaction mass with a stream of

nitrogen at 95° C. for 1½ hours, there were obtained 665 g. of a colorless viscous liquid with a chlorine content of 54.2%. Characteristics:  $n_D^{20}=1.578$ ;  $d_4^{20}=1.440$ .

*Example 5*

By chlorinating 410 g. of dodecyl benzene in the dark, at a temperature from 120 to 125° C., and with a rate of flow of chlorine of 24 l./hr., 843 g. of a reddish brown solid with a chlorine content of 55.0% were obtained after 22 hours.

*Example 6*

The operation was carried out as indicated in Example 1, using as starting material an alkyl benzene fraction boiling between 160° and 240° C., in which the number of carbon atoms of the alkyl chains varied between 5 and 11. By chlorinating in the dark with a rate of flow of chlorine of 30 l./hr. for 15 hours, and then of 20 l./hr., at a temperature between 115 and 120° C., there was obtained after 37 hours a limpid viscous liquid which was yellowish in color and had a chlorine content of 54.7%.

*Example 7*

For the purpose of studying its extreme-pressure characteristics in a lubricant, the product obtained in Example 1 was diluted, on the one hand, in a naphthene type oil known as "SHELL carnea 21" (trademark) and, on the other hand, in a paraffin type oil known as "350 Neutral" (trademark), which designates a lubricating grease obtained by distillation of petroleum, and of which the Saybolt viscosity at 37.8° C. is 350; the dilution rate was such that the chlorine content in each of the oils was 2.64% (i.e. about 4.7 g. of adjuvant in 100 g. of mixture).

The following table shows the rates of wear which were found, as a function of the pressure, after measurement on the 4-ball machine. By way of comparison, two other tests were carried out under exactly the same conditions as above, but with a chlorinated paraffin, used in the same quantity, in place of the chlorinated additive according to the invention.

| Pressure<br>(in kg.) | Wear (in mm.)                                 |                 |                      |                   |
|----------------------|-----------------------------------------------|-----------------|----------------------|-------------------|
|                      | Chlorinated alkyl benzene<br>of the invention |                 | Chlorinated paraffin |                   |
|                      | Naphthene<br>oil                              | Paraffin<br>oil | Naphthene<br>oil     | Paraffin<br>oil   |
| 60                   | 0.50                                          | 0.20            | 0.60                 | 0.45              |
| 100                  | 0.60                                          | 0.55            | 0.90                 | 0.60              |
| 150                  | 1.15                                          | 0.80            | 1.50                 | 1.30              |
| 180                  | 1.60                                          | 1.25            | 2.10                 | 1.70              |
| 200                  | 1.70                                          | 1.50            | 1 <sup>1</sup> 90    | 1 <sup>1</sup> 85 |
| 240                  | 2                                             | 1.85            | -----                | -----             |
|                      | 1 <sup>2</sup> 50                             |                 |                      |                   |

<sup>1</sup> Seizing at (kilograms).

*Example 8*

The operation was carried out under the same dilution conditions as in Example 7, using as additive the 54.2% chlorinated alkyl benzene obtained according to Example 4. The tests carried out on the 4-ball machine showed in this case the results set out in the following table, for each of the two oils, naphthene oil and paraffin oil, with 4% of additive.

| Pressure (in kg.) | Wear (in mm.)    |                  |
|-------------------|------------------|------------------|
|                   | Naphthene oil    | Paraffin oil     |
| 75                | 0.50             | 0.50             |
| 100               | 0.55             | 0.65             |
| 150               | 1.20             | 1.20             |
| 200               | 1.55             | 1.55             |
| 270               | 2.20             | 1.80             |
| 300               | ( <sup>1</sup> ) | ( <sup>1</sup> ) |

<sup>1</sup> Seizing.

*Example 9*

The operation was carried out as indicated in Example 7, with the same proportions of chlorine and the same oils, but using 54.7% chlorinated alkyl benzene as addi-

tive, this being prepared according to Example 6. The results obtained were:

| Pressure (in kg.) | Wear (in mm.) |              |
|-------------------|---------------|--------------|
|                   | Naphthene oil | Paraffin oil |
| 75                | 0.65          | 0.45         |
| 100               | 0.70          | 0.50         |
| 150               | 1.00          | 0.60         |
| 180               | 1.60          | 1.50         |
| 240               | 2.10          | 2.10         |

*Example 10*

Comparative tests were carried out on the 4-ball machine by dilution in a naphthene oil, under the same conditions as in Example 1, firstly the 55% chlorinated dodecyl benzene of the above Example 5 (product A) and on the other hand the 30% chlorinated dodecyl benzene (product B), which is already known for its extreme-pressure properties.

The 30% chlorinated hydrocarbon was used in a proportion clearly higher than that of the 55% chlorinated product, so as to have, after the same rates of dilution in the oil, equal contents of chlorine (2.50%).

The results as indicated in the following table were obtained:

| Pressure | Wear (in mm.)    |                  |
|----------|------------------|------------------|
|          | Product A        | Product B        |
| 75       | 0.50             | 0.50             |
| 100      | 0.60             | 0.60             |
| 150      | 0.82             | 0.96             |
| 180      | 1.0              | 1.50             |
| 200      | 1.25             | 1.95             |
| 250      | 1.75             | 2.45             |
| 280      | 2.0              | ( <sup>1</sup> ) |
| 320      | ( <sup>1</sup> ) | -----            |

<sup>1</sup> Seizing.

Apart from the fact that it is necessary to use larger quantities of 30% chlorinated dodecyl benzene so as to have the same final chlorine content in the oil, it has to be noted that the characteristics of this chlorinated hydrocarbon (product B) are clearly inferior to those shown by product A according to the invention.

*Example 11*

The chloralkyl benzene with 52.8% of Cl, obtained according to Example 3, added to the paraffin lubricating oil "350 Neutral" at respective rates of 4% and 8% by weight, showed the following results as regards wear:

| Pressure (in kg.) | Wear (in mm.) |      |
|-------------------|---------------|------|
|                   | 4%            | 8%   |
| 100               | 0.50          | 0.40 |
| 150               | 0.75          | 0.65 |
| 170               | 1.80          | 0.85 |
| 200               | 2.0           | 1.0  |

*Example 12*

The present example is given to serve as comparison with the modification of the invention illustrated by Example 13. It concerns a resinous polychlorobenzene polysulphide containing 19% of sulfur and 49% of chlorine, which belongs to the group of additives for lubricating greases described in French Patent No. 1,339,529.

This polysulphide was prepared in the following way: 20 g. of  $AlCl_3$  were added to 817 g. of a mixture comprising 30% of trichloro-1,2,3-benzene, 65% of trichloro-1,2,4-benzene and 5% of tetrachloro-1,2,4,5- and -1,2,3,4-benzenes; 405 g. of  $S_2Cl_2$ , previously diluted with 363 g. of the same trichlorobenzenes and tetrachlorobenzenes as indicated above, are progressively introduced over a period of 2 hours into the well stirred mixture, brought to 45° C. The total mixture then was kept at 45° C., while stirring, for half an hour, after which it was heated to 80° C. for 2 hours. The product of the reaction was then poured into water; the elimination of the  $AlCl_3$  was obtained by washing with dilute HCl, followed by a washing

with a dilute solution of sodium carbonate, then washing operations with water until neutral. The organic phase, after decantation of the aqueous phase, was subjected to a distillation at 20 mm. Hg until its temperature had reached 195 to 200° C. Thus, 260 g. of trichlorobenzenes were eliminated and there were recovered 950 g. of resinous polychlorobenzene polysulphides containing 49% by weight of Cl and 19% by weight of S.

This substance was tested as an additive to the "350 Neutral" oil under the same conditions as in Examples 7 to 11; for proportions of additive of 4% and 8% by weight, there were respectively found:

| Pressure (in kg.) | Wear (in mm.) |      |
|-------------------|---------------|------|
|                   | 4%            | 8%   |
| 100               | 0.65          | 0.45 |
| 150               | 1.15          | 1.20 |
| 170               | 1.50          | 2.10 |
| 180               | 2.01          |      |

#### Example 13

A mixture was prepared by adding 15 parts by weight of polychlorobenzene polysulphide according to Example 12 and containing 19% of S and 49% of Cl to 85 parts by weight of polychloroalkyl benzene with 52.8% of Cl, obtained according to Example 3. This 15/85 mixture of the 2 additives was tested as additive to the "350 Neutral" oil under the same conditions as above. The following respective wear values were found with contents of 4% and 8% by weight of this composite additive.

| Pressure (in kg.) | Wear (in mm.) |       |
|-------------------|---------------|-------|
|                   | 4%            | 8%    |
| 100               | 0.45          | 0.4   |
| 150               | 0.70          | 0.65  |
| 170               | 1.60          | 0.75  |
| 200               | 1.90          | 1.0   |
| 250               |               | 2.0   |
| 320               | (1)           | 2.30  |
|                   |               | 2.350 |

<sup>1</sup> Seizing. <sup>2</sup> Seizing above (kilograms).

These results are clearly better than those of each of Examples 11 and 12.

#### Example 14

Tests similar to those of Example 13 were carried out with a 25/75 composite additive, that is to say, a mixture of 25 parts by weight of the same polychlorobenzene polysulphide with 75 parts of the same polychloroalkyl benzene as in the preceding example.

The wear values were then:

| Pressure (in kg.) | Wear (in mm.) |       |
|-------------------|---------------|-------|
|                   | 4%            | 8%    |
| 100               | 0.40          | 0.35  |
| 150               | 0.65          | 0.55  |
| 170               | 1.50          | 0.70  |
| 200               | 1.80          | 1.00  |
| 250               |               | 2.00  |
| 320               | 2.10          | 2.20  |
|                   |               | 2.350 |

<sup>1</sup> Seizing above (kilograms).

These results, even better than those of Example 13, show that the proportion of 25/75 between the polysulphide and the polychloroalkyl benzene is more favorable than 15/85. There is a genuine synergistic effect between the two constituents, since the mixture thereof has an action on the lubrication which is clearly superior to

that of each of the constituents taken separately, as is the case in Examples 11 and 12.

The chlorinated alkyl benzenes used in the examples were stabilized beforehand, as indicated in the foregoing description. The thermal stability at 140° C., in the presence of iron and copper, was very good after one week. The resistance to water was excellent and in addition no trace of corrosion was observed with metals such as steels, copper and cast iron. The results of the examples which have been described show that the additives according to the invention have practically the same activity in the naphthene oils and the paraffin oils. These results are always better than those which are obtained when other chlorinated additives of known type are used.

On the other hand, it is apparent that the action of the additives according to the invention can be greatly improved by the addition of polysulphides of resinous polychloroalkyls; the mixed additives formed in this way have a more favorable effect on the lubrication than that which is achieved with each of the constituents taken separately.

We claim:

1. A lubricant composition containing, as a principal lubricating constituent, a lubricating oil and from 0.2 to 20% by weight of the composition of an extreme pressure lubricant additive comprising a mixture of from 10 to 90 parts by weight of a chlorinated alkyl benzene having a chlorine content of from 50 to 75% by weight, at least 75% of the chlorine content of said additive being bound to alkyl carbon atoms and at least one of the chloroalkyl radicals of the said additive having from 5 to 30 carbon atoms, and from 90 to 10 parts by weight of a resinous polychlorobenzene polysulphide soluble in hydrocarbon oils and containing from 15 to 25% sulfur and 44 to 55% chlorine.

2. The lubricant composition as defined in claim 1, which contains from 2 to 10% of the extreme pressure lubricant additive, and in which the chlorinated alkyl benzene constituent thereof has a chlorine content of from 52 to 60% by weight.

3. The lubricant composition as defined in claim 1, in which the extreme pressure lubricant additive comprises from 75 to 85% by weight of said chlorinated alkyl benzene and from 15 to 25% by weight of said resinous polychlorobenzene polysulphide, and in which the resinous polychlorobenzene polysulphide is soluble in paraffinic oils and contains about 15% sulfur and 49% chlorine.

4. The lubricant composition as defined in claim 1, in which the lubricating oil is a naphthenic base oil or a paraffinic base oil.

50

#### References Cited

##### UNITED STATES PATENTS

|           |        |                |             |
|-----------|--------|----------------|-------------|
| 2,121,824 | 6/1938 | Prutton        | 252—58      |
| 2,208,161 | 7/1940 | Prutton et al. | 252—48.8    |
| 3,175,972 | 3/1965 | Mitacek et al. | 252—48.8 XR |
| 3,179,592 | 4/1965 | Smith et al.   | 252—58      |

##### FOREIGN PATENTS

|    |           |        |         |
|----|-----------|--------|---------|
| 60 | 1,335,514 | 6/1963 | France. |
|----|-----------|--------|---------|

##### OTHER REFERENCES

Hugel "Erdol V. Kohle," vol. 8 (1955), pp. 651—655 (TN 860 E 7).

65 DANIEL E. WYMAN, Primary Examiner.

W. H. CANNON, Assistant Examiner.

UNITED STATES PATENT OFFICE  
CERTIFICATE OF CORRECTION

Patent No. 3,572,119

March 5, 1968

Bernard Demoures et al.

It is certified that error appears in the above identified patent and that said Letters Patent are hereby corrected as shown below:

In the heading to the printed specification, lines 5 to 7, for "Bernard Demoures, 14 Quai Jayr, Rhone, Lyon, France, and Gérard Schneider, 119 Quai Clemenceau, Rhone, Caluire, France" read -- Bernard Demoures, Lyon, France, and Gérard Schneider, Caluire, France, assignors to Societe Progil, Paris, France --.

Signed and sealed this 22nd day of July 1969.

(SEAL)

Attest:

Edward M. Fletcher, Jr.

Attesting Officer

WILLIAM E. SCHUYLER, JR.  
Commissioner of Patents